

## 1

3,139,334

 ATOMIZED LEAD-ALUMINUM ALLOY  
POWDER ARTICLE

Fritz Victor Lenel, Rensselaer, N.Y., assignor to Lead Industries Association, Inc., New York, N.Y., a non-profit corporation of New York  
No Drawing. Filed Sept. 29, 1961, Ser. No. 141,577  
1 Claim. (Cl. 75—5)

This invention relates to lead-base alloys having high strength and resistance to creep, and adequately high ductility.

Pure lead is soft and weak; its rate of creep at room temperature is so high that in many applications lead cannot be used as a structural material in itself. The strength and creep resistance of lead can be somewhat improved by alloying, particularly if the alloying element causes precipitation hardening as in conventional lead-antimony and lead-calcium alloys.

In precipitation hardening, an alloying element is added to the lead, which has higher solid solubility at temperature near its melting point than at room temperature. The alloy is rapidly cooled from the high temperature and then aged.

However, the extent to which lead can be strengthened and made more creep resistant by this type of alloying is limited. For instance, at 86° F. antimonial lead containing 6% Sb, has a creep rate of 1% in one year at a stress of 400 p.s.i.; and of 100% in one year at a stress of 860 p.s.i. An age hardened lead-calcium alloy with 0.03% Ca has creep resistance similar to the antimonial lead alloys.

In contrast, one of the lead base alloys according to the present invention, containing 0.55% aluminum, has, at 77° F., a creep rate of less than 0.5% in one year at a stress of 2500 p.s.i.; such alloy also has adequate tensile properties and ductility.

The preferred properties of prior art age hardened lead-base alloys are obtained by choosing a suitable chemical composition for the alloy and then giving the alloy an appropriate mechanical and thermal treatment. For the alloys according to the invention it is also necessary to choose a suitable chemical composition and appropriate mechanical and thermal treatments.

In contrast to most conventional alloys, the alloys according to the invention are fabricated by atomizing them into a fine powder, then compacting the powder, and then extruding the powder compact.

It has also been previously proposed to strengthen lead by atomizing it into a lead powder, then compacting it and working the compact. The dispersion of the lead oxide present in the powder strengthens the lead but such lead is so brittle as to be impractical for many uses.

It is an object of the invention to provide a lead base alloy article having greater resistance to creep and having also high strength and adequate ductility. Other objects of the invention will be more apparent from the following description and claim.

A preferred method of producing the alloy of the invention is described in the following, for two lead-aluminum alloys containing 0.55 and 1.7 weight percent of aluminum respectively, the remainder all lead.

## 2

The alloy is melted in a suitable crucible and heated to a temperature high enough to dissolve all the aluminum in the liquid lead. This temperature is in the range of 1500° to 1800° F. The melting point of lead is 621° F. and the melting point of aluminum is 1219.4° F.

The molten alloy is then atomized in the following manner:

A thin stream of the molten alloy is produced by pouring it through a suitable nozzle. This stream of metal is broken up into very fine droplets by impinging a stream of air of suitable velocity upon the stream of molten metal. The droplets of molten alloy freeze into powder particles.

The resultant powder is collected in a suitable container and sifted through a 325 mesh sieve. Only that portion of the powder, finer than 325 mesh (less than 44 microns) is used in the preparation of the alloy.

The powder is compacted in the atomized (as-received) condition. No compacting was done on "reduced" powder since it has been found that by the hydrogen-loss test, no readily reducible oxides exist in these powders. This is discussed more at length below.

The as-received powder is cold compacted into a compact 1 inch in diameter in a steel die under a pressure of 35,000–40,000 p.s.i. The resultant compact has a density of 98–99% of the density calculated by the rule of mixtures for a completely dense 99.45% Pb–0.55% Al alloy. The compact is extruded by indirect extrusion into a wire 0.156 inch in diameter at a temperature in the range 300° to 450° F.

It should be understood that the above method of consolidating the powder into a solid shape is only one of several methods which may be used to produce a solid shape. For instance, the lead powder may be fed into a rolling mill and rolled into a sheet. Cold rolling the powder into a sheet, and then hot re-rolling the sheet in the same temperature range as used for extrusion, results in rolled sheet having properties similar to those for the extrusions described below.

The preferred alloy composition is 99.45% lead–0.55% aluminum. This alloy composition and other lead-aluminum alloys have been tested in the form of extrusions, 0.15 inch in diameter. The tensile properties and the creep rate has been determined for extrusions made from as-received powder at extrusion temperatures as follows.

The data obtained are shown in Tables I to V below:

TABLE I

Mechanical Properties of As-Received Lead Powder at Various Extrusion Temperatures

[Characterized by severe embrittlement]

| Test   | Powder      | Extrusion Temperature, ° F | Tensile Strength, p.s.i. | Percent Elongation in 1 inch |
|--------|-------------|----------------------------|--------------------------|------------------------------|
| 55     |             |                            |                          |                              |
| A----- | Pb–PbO----- | Room Temperature.          | 7,690                    | 5.2                          |
| B----- | Pb–PbO----- | 200                        | 7,950                    | 6.6                          |
| C----- | Pb–PbO----- | 300                        | 6,660                    | 7.1                          |
| D----- | Pb–PbO----- | 400                        | 5,840                    | 11.6                         |
| E----- | Pb–PbO----- | 500                        | 5,120                    | 15.6                         |

**3**  
**TABLE II**

*Creep Stresses of Various Rolled Lead Alloys and of 95% Lead-5% Copper Powder Extrusions Compared to 99.45% Lead-0.55% Aluminum Powder Extrusion*

| Test | Alloy                           | Temperature, °F. | Steady State Creep Rate, Percent/year | Creep Stress, p.s.i. |
|------|---------------------------------|------------------|---------------------------------------|----------------------|
| A    | 6% Antimonial Lead              | 86               | 100                                   | 860                  |
| B    | Chemical Lead                   | 86               | 100                                   | 700                  |
| C    | Common Lead                     | 86               | 100                                   | 730                  |
| D    | 95% Pb-5% Cu Powder Alloy       | 77               | 113                                   | 4,050                |
| E    | 99.45% Pb-0.55% Al Powder Alloy | 77               | less than 0.5                         | 2,500                |

Test D in Table II refers to copper-lead powder alloys as disclosed in copending application Ser. No. 99,995, filed April 3, 1961, in the names of Schrade F. Radtke and Fritz V. Lenel.

**TABLE III**

*Mechanical Properties of As-Received Lead-Aluminum Powder Extrusions With Varying Amounts of Aluminum*

| Test | Weight, Percent Aluminum | Extrusion Temperature, °F. | Tensile Strength, p.s.i. | Percent Elongation in 1 inch |
|------|--------------------------|----------------------------|--------------------------|------------------------------|
| A    | 0.55                     | 450                        | 5,420                    | 20.0                         |
| B    | 1.7                      | 450                        | 3,680                    | 28.0                         |

**TABLE IV**

*Steady-State Creep Rate of the Alloy of Lead With 0.55% Aluminum at 77° F.*

[Extrusion temperature 450° F.]

| Test | Stress, p.s.i. | Steady-state Creep rate, Percent/year |
|------|----------------|---------------------------------------|
| A    | 2,000          | Less than 0.5                         |
| B    | 2,500          | Less than 0.5                         |
| C    | 3,000          | 1.8                                   |
| D    | 3,200          | 3.1                                   |

**TABLE V**

*Steady-State Creep Rates of the Alloy of Lead With 1.7% Aluminum at 77° F.*

[Extrusion temperature 450° F.]

| Test | Stress, p.s.i. | Steady-state Creep rate, Percent/year |
|------|----------------|---------------------------------------|
| A    | 2,500          | 1.1                                   |
| B    | 2,960          | 2.9                                   |

A practical use of this invention is for lead products which require resistance to creep, either at room or at slightly elevated temperatures. For radiation protection, lead may be extruded into bricks or into other products. For example, the extruded products may be used in lead-steel or lead-concrete sandwich structures, which must keep close dimensional tolerances. The design of these bricks or structures has heretofore been dictated by creep properties of the lead, rather than by its radiation protection. Simpler, lighter and lower cost structures are possible with a lead alloy according to the invention having improved creep resistance.

Very similar considerations apply to the use of lead or lead linings for corrosion protection in the chemical industry.

Lead-aluminum alloys have an advantage over lead-copper alloys in applications where shielding against neu-

**4**

tron radiation is involved, because aluminum has a very low capture cross-section for neutrons and is therefore not apt to produce secondary radiation when irradiated with neutrons.

It is believed that the improved strength and creep resistance of the lead alloys according to this invention is due to their structure, which consists of a very fine dispersion of particles of aluminum in the lead matrix of the powder particles. In order to produce such a structure it is necessary to cool the lead-aluminum alloy rapidly from a temperature at which the aluminum is in solution, i.e. well above the melting point of lead, to the vicinity of room temperature.

The strength and creep resistance of the alloy will depend upon the degree of dispersion of the aluminum particles in the particles of powder; the finer the dispersion, the stronger and more creep resistant the alloy. The degree of aluminum dispersion in the particles of powder will in turn depend on the rate of cooling of the alloy from the temperature where the aluminum is in solution. The finer the particles of powder, the faster the rate of cooling. It is therefore desirable to use quite fine powder.

Work has also been done on powders of different particle size. Even though best results have been obtained with powder, all of which is below 44 microns, good results have been obtained with powders of larger particle size.

In contrast to the lead-copper alloy powders the lead-aluminum alloy powders have a very low "hydrogen loss." The hydrogen loss is the percent loss in weight of a sample when it is heated in hydrogen at a certain temperature for a certain time (1020° F. for 30 minutes for lead). It is therefore an indication of the amount of oxide which can be readily reduced by hydrogen under the given reducing conditions. In lead-copper powders the hydrogen loss is due to the presence of lead oxide, or possibly of copper-oxide, which can be readily reduced by hydrogen. The low hydrogen loss in lead-aluminum powders means that no readily reducible oxides exist in these powders.

It is possible that any oxygen in the alloy reacts with the aluminum during atomizing and forms aluminum oxide. Since  $Al_2O_3$  cannot be reduced under the conditions of the hydrogen loss test, the "hydrogen loss" is low. It is possible that a considerable portion, or possibly even all, of the aluminum in the lead-aluminum powder is in the form of aluminum oxide.

It is not inconceivable that the higher creep-resistance of the lead-aluminum powder extrusions, compared with the lead-copper powder extrusions, is due to the fact that aluminum oxide is a more effective strengthener than metallic copper or that the aluminum oxide is more finely divided in the lead than the metallic copper. It is also possible that the higher strength and creep resistance of the alloy with 0.55% Al compared with those of the 1.7% Al is due to the form in which the aluminum is which the aluminum is present (metallic aluminum vs. aluminum oxide) or due to the distribution of the aluminum or its oxide (coarse vs. fine).

Work has also been done to determine the range of composition of the Pb-Al alloys, which have these desirable properties. This work indicates that the aluminum content should run from 0.1% to 2.0% aluminum by weight, remainder lead.

What is claimed is:

A worked lead base powder article, the particles of said powder being obtained by atomizing a molten lead-aluminum alloy in which the aluminum is completely dissolved in the lead, said particles consisting of a fine dispersion in a lead matrix of a form of aluminum selected from the group consisting of aluminum and aluminum oxide, and said lead-aluminum alloy, before atomizing, consisting essentially of from 0.1 to 2.0% by weight of aluminum with the balance lead, said article being formed by pressure compacting said particles and working the

resulting compacted form, said article having a substantially lower creep rate than that of pure lead.

**References Cited** in the file of this patent

UNITED STATES PATENTS

- |           |                 |                |
|-----------|-----------------|----------------|
| 1,635,653 | Williams        | July 12, 1927  |
| 1,761,506 | Williams        | June 3, 1930   |
| 2,156,802 | Cooper          | May 2, 1939    |
| 3,053,654 | McKim           | Sept. 11, 1962 |
| 3,085,319 | Giraitis et al. | Apr. 16, 1963  |

5

10

FOREIGN PATENTS

- |         |               |              |
|---------|---------------|--------------|
| 821,336 | Great Britain | Oct. 7, 1959 |
|---------|---------------|--------------|

OTHER REFERENCES

- |    |                                                                                                                         |
|----|-------------------------------------------------------------------------------------------------------------------------|
| 5  | Campbell et al.: "The Alloys of Aluminum and Lead," Canadian Journal of Research, vol. 18, sec. B, 1940, pages 281-287. |
|    | Claus et al.: "Zur Kenntnis der Systeme Al-Pb-Cu und Al-Pb," Metallwirtschaft, 18, 1939, pages 957-960.                 |
| 10 | Hansen: Constitution of Binary Alloys, 2nd ed., 1958, McGraw-Hill Book Company, Inc., N.Y., pages 122-124.              |